

## UNITED STATES PATENT OFFICE

BERNHARD SCHARNOW, OF BERLIN-CHARLOTTENBURG, GERMANY, ASSIGNOR TO  
DEUTSCH-ATLANTISCHE TELEGRAPHENGESELLSCHAFT, OF BERLIN, GERMANY

## FERROMAGNETIC MATERIALS

No Drawing. Application filed April 21, 1930, Serial No. 446,168, and in Germany December 10, 1928.

This invention relates to magnetic alloys of the nickel-iron class having a high permeability at low magnetizing forces, such as used for loading telephone and telegraph 55 conductors or the like in electrical circuits.

It aims to increase the constancy of permeability in low magnetizing fields by increasing the small coercivity of such metals without unduly impairing the general high 10 order of initial permeability, so as to improve their character and applicability to the stated and other uses as will be better understood from the following description.

Chief among the properties required in alloys of this kind are:—(a) high initial permeability, and (b) a relatively small change in permeability throughout the largest possible range of small field strengths. Condition (b) is fulfilled by an alloy having a 15 comparatively high coercivity, since it is well known that the higher the coercivity of alloys of a certain class becomes, the less the dependence of the permeability on the strength of field at small magnetizing forces. 20 In the following description therefore, the amount of the coercivity will be taken as an inverse measure of the change of the permeability with strength of field.

It is well known that pure nickel-iron alloys, especially those having approximately 30 80% nickel content possess an extraordinarily high initial permeability, but these suffer a relatively great change of permeability with changing strength of field. Other alloys, such as those consisting for example of cobalt, iron and nickel, show an extraordinarily small increase of permeability with varied strength of field and accordingly satisfy the above-mentioned condition (b). 35 However, with these last-mentioned alloys there is a limit to the magnitude of initial permeability, which limit renders the alloy 40 unsuitable for many purposes.

The present invention provides a generally 45 applicable method of procedure which, in the case of nickel-iron alloys of high initial permeability and small coercivity makes it possible to increase the coercivity and thereby 50 to decrease the change in permeability, without unduly lowering the value of the initial

permeability. It embodies a process in the manufacture or thermal production of alloys with finely distributed heterogeneous constituents, the term "heterogeneous" as opposed to mixed crystal being intended to be 55 understood in the sense known and fixed by definition in metallography. Said process moreover enables alloys with any desired properties to be systematically produced.

Hitherto it has been considered desirable, 60 if not essential, that the ingredients in highly magnetic mechanically-workable nickel-iron alloys should be completely in solid solution, and when additional elements have been proposed either to increase the initial permeability or the specific resistance, or else to render mechanical treatment easier, their nature and amount have been selected so as to bring about their complete solid solution. 65 For example, manganese, chromium, cobalt, tungsten, copper, silicon, molybdenum and the like have been added to nickel-iron alloys in such proportions that all formed mixed crystals therewith. 70

The behavior of metals is of course known so far as the forming of mixed crystals, or solutions in each other is concerned. For instance, it is known that an alloy of nickel and iron is capable of taking up a considerable percentage of copper in the mixed crystals of nickel and iron. Only after a certain limit of copper addition is passed are parts of the copper found in the solid body as separate heterogeneous constituents. The conditions under which these constituents are 80 formed have been known for many materials, although tests have not been made for all the different metals and alloys. However, it was not known that heterogeneous constitution in nickel-iron alloys of high initial permeability might be used to achieve a special technical effect and create, so to speak, an inner "tension" causing an increase of the 85 coercivity of the metals. 90

The discovery of this fact led to this invention, according to which, as distinguished from prior knowledge and practice, there are produced in the high initial permeability alloys certain materials or elements such as 95 silver out of solid solution and disseminated 100

- in a finely divided state. A particular form of heat treatment is required to produce the desired result according to the invention, which heat treatment comprises heating the alloy, after working it to shape as desired, to an annealing temperature, e. g. 900° C. or above, then quenching it from that temperature, or from a somewhat lower temperature, e. g. 600° C., in order to obtain a condition of super-saturation of the added element in solid solution, and thereafter soaking the material at a temperature such as 300° to 500° C. for a sufficiently long time.
- 10 The separate or heterogeneous particles left in the material (whether they be of microscopic or sub-microscopic size) then set up a state of strain therewith owing to the difference of their thermal coefficients of expansion or to the occurrence of a change of volume, by which state of strain the coercivity of the material is increased. The initial permeability however is affected only within certain limits. The value of the initial permeability and of the coercivity may be varied by varying the nature and quantity of the added substance as well as by suitably varying the details of the heat treatment, and within limits any desired combination of both values can be obtained.
- 15 The coefficients of solubility of the individual substances with respect to each other are sufficiently known in science and engineering. Also if several substances are soluble in each other at very high temperatures, especially in the molten state, it is nevertheless known that many of them dis-associate again at lower temperatures, especially if assisted by heat treatment of suitable degree and extended over some length of time. Substances of this behavior are generally described as not readily forming mixed crystals.
- 20 In addition to silver as stated, examples of materials or elements which may be added to the high permeability metals or alloys for the stated purpose of increasing the coercivity thereof, arsenic, beryllium, boron, phosphorus, sulphur and zirconium are other possibilities. It is therefore immaterial which of the well known materials or elements is added to the metal or alloy so long as it has or shows, when used in comparatively small amounts, the special behavior of forming heterogeneous constituents which do not pass into or stay in solid solution at room temperature. Elements such as copper, which are comparatively soluble in the nickel-iron solid complex, cannot be usefully employed according to the present invention.
- 25 The following table shows the effect of annealing a nickel-iron alloy with an addition of silver, cooling rapidly from 600° C. and shows that the coercivity can be increased at will, while retaining a substantial
- 30
- 35
- 40
- 45
- 50
- 55
- 60
- 65

## Alloy 77.5% Ni, 20.5% Fe, 2.5% Ag

| State                        | Initial permeability | Coercivity | 70 |
|------------------------------|----------------------|------------|----|
| Rapidly cooled from 600° C.  | 5880                 | 0.16       |    |
| Aged for 1 hour at 350° C.   | 4812                 | 0.2        |    |
| Aged for 6 hours at 350° C.  | 4030                 | 0.29       |    |
| Aged for 11 hours at 350° C. | 4100                 | 0.32       |    |
| Aged for 16 hours at 350° C. | 3630                 | 0.35       |    |
| Aged for 21 hours at 350° C. | 3570                 | 0.37       |    |

75

Having thus described my invention, what I claim as new and desire to secure by Letters Patent of the United States is:—

1. The process of producing magnetic alloys of the nickel-iron class with high initial permeability and with reduced variation of permeability in small magnetic fields, characterized by incorporating in the alloy an additional element which does not readily form mixed crystals with the nickel-iron complex, heating the alloy and quenching it from a high temperature so as to obtain a condition of super-saturation of the element in solid solution and thereafter soaking the material at a lower temperature for a substantial period of time, in order to precipitate some of the element out of solution in a finely divided state.

80

2. The process of producing magnetic alloys of the nickel-iron class with high initial permeability and with reduced variation of permeability in small magnetic fields, characterized by incorporating in the alloy an additional element which does not readily form mixed crystals with the nickel-iron complex, heating the alloy to an annealing temperature, quenching so as to obtain a condition of super-saturation of the element in solid solution, and thereafter soaking the material between about 300° and 500° C. for a substantial period of time in order to precipitate some of the element out of solution in a finely divided state.

95

3. The process of producing magnetic alloys of the nickel-iron class with high initial permeability and with reduced variation of permeability in small magnetic fields, characterized by incorporating in the alloy an additional element which does not readily form mixed crystals with the nickel-iron complex, heating the alloy to an annealing temperature, cooling rather slowly to a lower temperature, such for example as 600° C., quenching so as to obtain a condition of super-saturation of the element in solid solution, and thereafter soaking the material between about 300° and 500° C. for a substantial period of time in order to precipitate some of the element out of solution in a finely divided state.

100

4. The process of producing magnetic alloys of the nickel-iron class with high initial permeability and with reduced variation of permeability in small magnetic fields, characterized by incorporating silver in the al-

110

115

120

125

120

loy, heating the alloy and quenching it from a high temperature so as to obtain a condition of super-saturation of the silver in solid solution, and thereafter soaking the material 5 between about 300° and 500° C. for a substantial period of time in order to precipitate silver out of solid solution in a finely divided state.

5. The process of producing magnetic alloys of the nickel-iron class with high initial permeability and with reduced variation of permeability in small magnetic fields, characterized by incorporating silver in the alloy, heating to at least 900° C., quenching in order 10 to obtain a condition of super-saturation of the silver in solid solution, and thereafter soaking the material between about 350° and 400° C. in order to precipitate silver out of solid solution in a finely divided state.

20 6. The process of producing magnetic alloys of the nickel-iron class with high initial permeability and with reduced variation of permeability in small magnetic fields, characterized by incorporating silver in the alloy, 25 heating to at least 900° C., cooling rather slowly to a lower temperature, such for example as 600° C., quenching from that temperature in order to obtain a condition of super-saturation of the silver in solid solution, 30 and thereafter soaking the material between about 350° and 400° C. in order to precipitate silver out of solid solution in a finely divided state.

25 7. Process as claimed in claim 4, in which the amount of silver incorporated is between about 0.3% and 5%.

8. Process as claimed in claim 4, in which the amount of silver incorporated is about 2.5%.

40 9. A magnetic alloy of the nickel-iron class having a high initial permeability and relatively small variation of permeability in small magnetic field, characterized by comprising an additional element of a kind which does 45 not readily form mixed crystals with the nickel-iron complex, the said element being out of solid solution and disseminated in a finely divided state throughout the mass of the alloy.

50 10. A magnetic alloy of the nickel-iron class having a high initial permeability and relatively small variation of permeability in small magnetic fields, characterized by comprising silver out of solid solution and disseminated in a finely divided state throughout the mass of the alloy.

55 11. A magnetic alloy of the nickel-iron class having a high initial permeability and relatively small variation of permeability in small magnetic fields, characterized by comprising between 0.3% and 5% silver out of solid solution and disseminated in a finely divided state throughout the mass of the alloy.

12. A magnetic alloy of the nickel-iron

class having a high initial permeability and relatively small variation of permeability in small magnetic fields, characterized by comprising about 2.5% silver out of solid solution and disseminated in a finely divided state throughout the mass of the alloy. <sup>70</sup>

In testimony whereof I affix my signature.  
BERNHARD SCHARNOW.

75

80

85

90

95

100

105

110

115

120

125

130